

June 21, 1938.

M. BRAUN

2,121,393

METHOD FOR COPPERING OF SEAMLESS TUBES

Filed Nov. 18, 1935



Inventor:  
Matthäus Braun  
Emil Römelyche  
Attorney

## UNITED STATES PATENT OFFICE

2,121,393

## METHOD FOR COPPERING OF SEAMLESS TUBES

Matthäus Braun, Frankfort-on-the-Main,  
GermanyApplication November 18, 1935, Serial No. 50,450  
In Germany July 4, 1935

6 Claims. (Cl. 91—70.2)

The invention relates to coppered steel tubes as a satisfactory substitute for copper tubes, and to the coppering of finished seamless or welded steel tubes.

5 The galvanic coppering of finished tubes is not always applicable. It is attended by difficulties particularly in the case of narrow tubes in which an anode cannot be inserted because the distance between the anode and the wall of the tube would be too small. One is limited in this connection to a minimum distance of about 50 millimeters between anode and cathode so that only tubes of 10 100 millimeters bore and upwards can be satisfactorily coppered by galvanic methods.

15 The invention is illustrated on the accompanying drawing in which:

Figure 1 is a cross-sectional view of the steel tube with the copper coils therein and thereon,

20 Fig. 2 is a longitudinal sectional view of the tube of Fig. 1, and

Fig. 3 is a diagrammatic side view of the coppering apparatus.

According to the present invention a specially prepared steel tube is coated with copper in a melting furnace. The preparation consists, according to Fig. 1, in inserting a helically wound copper wire *b* in the steel tube *a* to be coppered. This wire of round cross section has its coils of outer diameter equal to that of the interior diameter of the steel tube. It is wound helically in order that it may be applied over its whole length closely against the inner wall of the steel tube and thus produce an uninterrupted metallic contact with the tube wall. In this manner during 25 the melting operation of the furnace, the copper will flow in such a manner that it will uniformly coat the whole inner wall of the steel tube because during the liquefying of the copper, close contact with the steel tube wall is ensured at 30 every place. If the outer wall of the tube is to be coppered, a similar procedure is adopted. This wall is wound with the copper wire helix *c*, the inner diameter of the coils of which correspond to the outer diameter of the steel tube. The flux 35 usually consisting of an aqueous solution of borax, is applied in liquid condition. Owing to adhesion, it will be retained in greater amount about the rounding of the wire and particularly in the seams between the tube wall and the line of contact of the wire therewith, than at the smooth surfaces. 40 Thereby the flux is brought to the very places where it is required.

The tube thus prepared is now brought into a furnace which has the melting temperature 45 of copper and which preferably contains a reduc-

ing atmosphere to avoid burning or oxidation. According to the thickness of the copper wire, the copper deposit may be increased or decreased whereby a thicker or a thinner coppering is obtained. The copper layer may thus have its thickness regulated by choosing a thinner or a thicker wire or by arranging the coils of the wire closer or farther apart. If an extremely scanty or 5 thinner copper coating is desired, the steel tube is traversed through the furnace in an oblique plane. 10 The copper wire liquefies and flows so that the whole wall surface, the inner or the outer wall, of the steel tube is uniformly coated and brought into close metallic contact with the copper. Only so much copper adheres to the wall as corresponds to the adhesion of the metals. The excess material owing to the oblique position of the tube flows downwards and away at the lower end of the same. In this manner an extremely thin metal coating is obtained. 15

20 In this process it must be taken into consideration that it is possible for a few porous places, even if very small ones, to form on the surface, for example by development of bubbles. To remove these the tube is subsequently subjected to a cold drawing operation. The coppered tube after 25 cooling is thus drawn from a larger to a smaller diameter and the copper coating is compressed molecularly in such a manner that it undergoes 30 a compacting of its surface which uniformly distributes the copper molecules and eliminates porous places.

35 This process can be further improved by giving the tube a rotary movement during the melting operation in the furnace. The tube should be rotated about its longitudinal axis.

40 By this rotation the metal of the copper wire helix inserted in the steel tube and brought to the melting point in the muffle of the melting furnace, is impelled against the inner wall of the tube and pressed against the same. The copper will be thereby distributed very uniformly and very finely over the whole inner wall. The centrifugal action obtained by the rotation of the 45 tube thus has the advantage that the flow of the copper from the tube wall takes place more uniformly and that the coating is denser. In particular, the rotary movement prevents accumulation of excess molten copper at the lower end of 50 the tube, owing to its oblique position, which would give a thicker coating at this end.

55 The speed of rotation of the tube in this operation is preferably between 1500—2000 revolutions per minute.

The finished copper tube can then be drawn as before to a smaller diameter.

In Fig. 3, the steel tube A which may be placed in any suitable position, is advanced obliquely through the muffle or chamber B of the furnace C in which it is to be coppered. It is not essential that the position should be oblique, it may be horizontal, but the oblique position is preferred. The copper wire helix is inserted into the interior of the tube. The tube A is given a rotary movement from the motor D. This motor is mounted on a slide F which is given a feed movement by means of a screw spindle or shaft G driven by a motor E. The tube while retaining its oblique position is thus advanced through the furnace with a speed which corresponds to the time required for the satisfactory melting of the copper in the chamber B. On its issue from the melting furnace, the copper tube is received upon suitable guide means, and withdrawn.

By suitable selection of the diameter of the copper wire helix and the number of its coils it is possible to determine with great precision the amount of copper required to produce a satisfactory copper coating of any desired thickness. Instead of the illustrated lathe mechanism for feeding and rotating the steel tube, other means for this purpose may be employed. For example, a whole series of tubes may be operated by rollers or sets of rollers some of which effect the feed movement while others effect the rotary movement.

It is of course understood that solid bars may be coppered in the same manner as tubes by first applying a copper wire helically around the outside of the bar and then passing this bar with the wire thereon through the furnace.

It is further to be understood that the process can be applied to any metallic article other than a tube and that any coating metal or alloy other than copper can be utilized as well as any melting method can be applied. Therefore, while the invention particularly concerns tubes, it is however understood that any metallic article may be coated provided the coating is carried out by applying the metallic wire closely or in intimate contact with the surface to be coated.

I claim as my invention:

1. A process of internally coppering tubes and the like comprising inserting in the tube copper wire wound in a helix of such diameter that the wire presses elastically along its whole length against the inner wall of the tube, applying a liquid flux to the tube and the wire helix wherein the flux will be retained to a greater amount around the wire of the helix, and subjecting the tube with the wire therein to heat to melt the copper and thus coat the inner wall.

2. A process of internally coppering tubes and the like comprising inserting in the tube copper

wire wound in a helix with widely spaced coils and of such diameter that the wire presses elastically along its whole length against the inner wall of the tube, applying a liquid flux to the tube and the wire helix wherein the flux will be retained to a greater amount around the wire of the helix, and subjecting the tube with the wire therein to heat to melt the copper and thus coat the inner wall. 5

3. A process of internally coppering tubes and the like comprising inserting in the tube copper wire wound in a helix of such diameter that the wire presses elastically along its whole length against the inner wall of the tube, applying a liquid flux to the tube and the wire helix wherein the flux will be retained to a greater amount around the wire of the helix, subjecting the tube with the wire therein to heat to melt the copper and thus coat the inner wall, and rotating the tube about its longitudinal axis during heating. 10 15 20

4. A process of internally coating metal tubes and the like with a lining of metal more fusible than that of the tube comprising inserting in the metal tube a wire of the more fusible metal wound in a helix the coils of which are at all points in self sustaining contact with the inner wall of the tubes, applying a liquid flux to the tube and the wire helix wherein the flux will be retained to a greater amount around the wire of the helix, and subjecting the tube with the wire therein to heat 30 35 40 sufficient to melt the wire and thus coat the inner wall with the more fusible metal. 50

5. A process of internally coating metal tubes and the like with a lining of metal more fusible than that of the tube comprising inserting in the metal tube a wire of the more fusible metal wound in a helix with widely spaced coils and the coils of which are at all points in self sustaining contact with the inner wall of the tube, applying a liquid flux to the tube and the wire helix wherein the flux will be retained to a greater amount around the wire of the helix, and subjecting the tube with the wire therein to heat sufficient to melt the wire and thus coat the inner wall with the more fusible metal. 45 55

6. A process of internally coating metal tubes and the like with a lining of metal more fusible than that of the tube comprising inserting in the metal tube a wire of the more fusible metal wound in a helix the coils of which are at all points in self sustaining contact with the inner wall of the tube, applying a liquid flux to the tube and the wire helix wherein the flux will be retained to a greater amount around the wire of the helix, subjecting the tube with the wire therein to heat sufficient to melt the wire and thus coat the inner wall with the more fusible metal, and rotating the tube about the longitudinal axis. 55

MATTHÄUS BRAUN.

60